

1

3,502,471

## NEW LIGHT-DEVELOPABLE PHOTOGRAPHIC MATERIAL AND RECORDING PROCESS

Paul Desire Van Pee, Edegem, and Jozef Frans Willems, Wilrijk-Antwerp, Belgium, assignors to Gevaert-Agfa N.V., Mortsel-Belgium, a Belgian company  
No Drawing. Filed Oct. 11, 1966, Ser. No. 585,731  
Claims priority, application Great Britain, Oct. 11, 1965,  
42,969/65  
Int. Cl. G03c 5/32

U.S. Cl. 96—45.2

22 Claims 10

### ABSTRACT OF THE DISCLOSURE

Photographic elements are defined which comprise a radiation-sensitive silver halide emulsion layer of the light developable type. The layer is applied from a coating composition containing a silver iodide sol and/or a compound which will release free iodide ions and a halogen acceptor corresponding to the formula or to a tautomeric structure thereof as follows:



wherein each of R<sub>1</sub>, R<sub>2</sub>, R<sub>3</sub>, R<sub>4</sub> and R<sub>5</sub> is hydrogen, an alkyl group or an aryl group, with the proviso, however, that at least one of the substituents R<sub>2</sub> and R<sub>3</sub> is hydrogen; R<sub>4</sub> and R<sub>5</sub> may also be the atoms necessary to complete a carbocyclic ring. These light-developable silver halide materials are useful in high-speed recording such as high-speed oscillographic recording of events which occur in rapid sequence, and the like.

The present invention relates to photographic elements comprising an improved light-developable radiation-sensitive silver halide emulsion layer, as well as to a process for making records employing said elements.

The light-developable silver halide materials have become of increasing interest, for they possess desirable properties for high speed recording, such as high speed oscillographic recording of events, which occur in rapid sequence, and the like.

Light-developable silver halide materials for direct recording are radiation-sensitive materials in which a visible image can be obtained, after an exposure to a high intensity source of radiation has been initially utilised to form a latent image, by an additional exposure to a radiation of lower intensity such as diffuse daylight or artificial light. The secondary exposure, also called latensification, is an overall exposure, including exposing the areas in which the initial latent image was formed as well as the surrounding background to an additional amount of radiation.

It is known that in general, intense exposure favours the formation of a latent image in the interior of the grains while low-intensity exposure forms almost exclusively a surface latent image. The surface latent image is the one developed by a usual chemical development whereas the internal latent image is practically not developed by such processing. The light absorbed by the silver halide in the secondary exposure provides the energy for the development of the internal latent image to a visible form (cf. H. Hunt High Speed Direct Recording Papers, Phot. Sci. Eng., vol. 5, No. 2, 1961).

2

Many of the known light-developable, radiation-sensitive materials have the disadvantage that on latensification the image becomes very slowly visible, that the background tends to darken fast and that the maximum density of the image decreases on a prolonged secondary exposure.

It has now been found that the addition of at least one member selected from a silver iodide sol and a compound that sets free iodide ions together with at least one halogen-acceptor corresponding to the following general formula or to a tautomeric structure thereof:



wherein each of R<sub>1</sub>, R<sub>2</sub>, R<sub>3</sub>, R<sub>4</sub> and R<sub>5</sub> represents a hydrogen atom, an alkyl group including a substituted alkyl group or an aryl group including a substituted aryl group, with the proviso, however, that at least one of the substituents R<sub>2</sub> and R<sub>3</sub> represents a hydrogen atom; R<sub>4</sub> and R<sub>5</sub> may also represent the atoms necessary to complete a carbocyclic ring including a substituted carbocyclic ring, to light-developable radiation-sensitive silver halide emulsions results unexpectedly and surprisingly in the production of a light-developable material in which an improved image can be obtained, showing a favourable contrast between the image and the background (i.e. having a good net density) and having a very good stability as well as a good chemical developability. As will be seen from the examples hereinafter, the effect of the simultaneous addition of the above compounds is much more important than the effects obtained on the one hand by the addition of the halogen acceptor alone and on the other hand by the addition of the silver iodide sol and/or the compound splitting off iodide ions alone. When only a member of one of these two groups of compounds is incorporated into the light-developable radiation-sensitive emulsion layer the difference between the maximum and minimum density is considerably lower than when both groups are present together. This additive effect is the more surprising since it was found that this effect could not be obtained in the case of a combination of a compound setting free iodide ions with many other generally known and often used halogen-acceptors e.g. hydrazothiocarbonamide, thiosemicarbazide and thiourea.

The improved light-developable radiation-sensitive photographic silver halide elements according to the present invention permit a rapid access to and prolonged examination of the image formed on photodevelopment and also permit a chemical development and fixing treatment in order to obtain permanent records of the traces or images. The material according to the present invention shows a high degree of sensitivity to the trace beam coupled with a highly stable background i.e. a background which is not very sensitive to low intensity radiation, thus resulting in a maximum contrast between the image and background. Thus, the images or traces obtained on light-development with elements according to the present invention are characterized by a high net density, i.e. an optimum contrast between the image and background, a good resistance to fogging of the non-image areas even when exposed for a long time to ambient lighting and even when no chemical development occurs. Of course, when the traces or images produced on latensification are exposed to ambient lighting for a long time the background darkens slowly, however, the contrast between image and background will remain for many hours. The

## 3

images or traces will not remain visible when permanently exposed to light. To keep a permanent record of the races or images, the material has to be chemically developed and fixed, preferably not too long after the light-development. Without said development and fixing step, the record will remain permanently only when the light-developed images are exposed to light infrequently and kept in the dark when not in use. Indeed, the image will last practically indefinite if protected from prolonged exposure to strong light.

Another advantage offered by the light-developable elements of the invention is that it is possible to carry out the light-development while supplying heat, whereby the recorded image becomes almost immediately visible for the reason that, when heating, it is possible to increase the light-intensity of the secondary exposure without producing fog. A probable explanation of this phenomenon has been given by Jacobs, Phot. Sci. & Eng., vol. 5, No. 1, 961. By the fact that when operating at elevated temperature a more rapid image access is obtained, it is not necessary in those instances where there is recorded at high writing speeds and thus at high paper transport speeds, to expose considerable meters of paper to ambient light at the same time, which would lead to a handling problem. Some oscilloscopes operate according to this principle: after the high-intensity exposure the print-out material is passed over a heated plate while being exposed to fluorescent U.V. lamps so that a visible image is produced almost immediately.

The following is a non-restrictive list of halogen acceptors, which have proved to be particularly suitable for use according to the present invention, and which correspond to the above general formula:

## Compound 1



6,6-dimethyl-3-thio-1,6-dihydro-as-triazine-3,5(2H,4H)-dione

Melting point: 248-249° C. Preparation described by Fusco and Rossi, Gazz. Chim. Ital. 89, 373 (1954).

## Compound 2



3-thio-1,2,4-triazaspiro[5,5]undecane-3,5-dione

Melting point: 224° C. Preparation described by Fusco and Rossi, Gazz. Chim. Ital. 89, 373 (1954).

## Compound 3



4,6,6-trimethyl-3-thio-1,6-dihydro-as-triazine-3,5(2H,4H)-dione

Melting point: 190° C. This compound can be prepared according to Preparation 1 as described further hereinafter.

## 4

## Compound 4



4-methyl-3-thio-1,2,4-triazaspiro[5,5]undecane-3,5-dione

Melting point: 210° C. This compound can be prepared according to Preparation 2, as described further hereinafter.

## Compound 5



1-phenyl-4-methyl-3-thio-1,6-dihydro-as-triazine-3,5(2H,4H)-dione

Melting point: 180-190° C. This compound can be prepared according to Preparation 3, as described further hereinafter.

## Compound 6



1-phenyl-3-thio-1,6-dihydro-as-triazine-3,5(2H,4H)-dione

Melting point: 172-173° C. Preparation described by Busch and Meussdörffer, Ber. 40, 1021 (1907).

## Compound 7



1-methyl-4-ethyl-3-thio-1,6-dihydro-as-triazine-3,5(2H,4H)-dione

Melting point: 129° C. This compound can be prepared according to Preparation 4 as described further hereinafter.

## PREPARATION 1

A. Preparation of the intermediate product 1-(1'-cyano-1'-methyl-ethyl)-4-methylthiosemicarbazide

21 g. of 4-methyl thiosemicarbazide are dissolved in 80 ccs. of a mixture of ethanol and water (1:1). Whilst stirring the solution, there are successively added at room temperature: 11.5 ccs. of acetic acid, a solution of 13 g. of potassium cyanide in 25 ccs. of water and 12.6 ccs. of acetone. The reaction mixture is refluxed for 1 hour. After cooling, the crystals formed are filtered by suction (yield: 34.5 g.—melting point: 197-203° C.) and recrystallized from 1600 ccs. of ethanol.

Yield: 25.5 g. 1-(1'-cyano-1'-methyl-ethyl)-4-methylthiosemicarbazide. Melting point: 210° C.

Microanalysis.—Calculated for C6H12N4S, molecular weight: 172 (percent): C, 41.90; H, 7.03; S, 18.64.

75 Found (percent): C, 42.45; H, 6.87; S, 18.39.





Organic compounds with labile iodine atom which have proved to be suitable for use according to the invention are for instance mono-iodo-acetic acid and 4-iodo-butane sulphonic acid potassium salt.

Finally, as regards the onium chloroiodates there can be referred to Belgian patent specification No. 515,895 filed Nov. 29, 1952 by Gevaert Photo-Producten N.V.; examples of suitable onium chloroiodates are among others more particularly:



Instead of or in addition to a compound setting free iodide ions, a silver iodide sol comprising an appropriate protective colloid can be added with the same effect to the silver halide emulsion. A very suitable silver iodide sol can be prepared by slowly adding while strongly stirring the following solution A to the following solution B, both solutions being heated to 35° C.

Solution A:

3NAgNO<sub>3</sub>.—17 ccs.  
water up to 1 litre

Solution B:

3NKI.—17 ccs.  
gelatin.—40 g.  
water up to 1 litre

The amount of compound setting free iodide ions may also vary within very wide limits. In general an amount from about 0.01 g. to about 20 g. preferably from about 0.1 g. to about 5 g. per mole of silver halide is applied. The same applies to the limits within which the silver iodide sol is used. In the latter case the above amounts relate to the silver iodide and not to the total sol. The addition of a member selected from a silver iodide sol and at least one compound setting free iodide ions, and

preferably also the addition of the halogen-acceptor occurs after the emulsion preparation and preferably just before coating on a suitable support. Except the addition of the silver iodide sol, any other addition can occur from a solution of the compound involved in a suitable solvent, which is mostly water but may also be an organic solvent.

By the addition to a silver halide emulsion of a compound setting free iodide ions or of a silver iodide sol, 10 silver iodide is produced on the surface of the silver halide grains of the emulsion, in the former case by conversion and in the latter by adsorption. The formation of silver iodide at the surface of the grains and the favourable effects resulting therefrom for the method of 15 the present invention can also be attained by conducting the emulsion layer obtained after coating through a solution, preferably an aqueous solution of a compound setting free iodide ions, or by treating this emulsion layer in some other way therewith.

20 According to the invention any silver halide emulsion of the light-developable type may be used. These kinds of emulsions are very well known to those skilled in the art. They mainly or entirely form an internal latent image and only to a little extent an external latent image.

25 A silver halide emulsion that mainly or entirely forms an internal latent image and only to a little extent an external latent image is an emulsion in which only few or no exposed grains at all are developable into silver by a developing solution that cannot act as a developer for 30 a latent image inside the grains i.e. a so-called "surface" developer, such as:

p-Hydroxyphenyl glycine—10 g.  
Sodium carbonate (cryst.)—100 g.  
Water to 1000 ccs.

35 and wherein the exposed grains are well developable to silver by a developing solution that acts as a developer for latent image inside the grains i.e. a so-called "internal" developer such as the following solution:

40 Hydroquinone—15 g.  
Monomethyl-p-aminophenol sulphate—1.5 g.  
Sodium sulphite (anhydrous)—50 g.  
Potassium bromide—10 g.  
Sodium hydroxide—25 g.  
45 Sodium thiosulphate (cryst.)—20 g.  
Water to 1000 ccs.

By a silver halide emulsion that mainly forms internal 50 latent image and little external latent image there is more particularly meant a silver halide emulsion, a test layer of which upon exposure to a light intensity scale for a fixed time between  $\frac{1}{100}$  and 1 sec. and development for 3 min. at 20° C. in the above "internal" developer, exhibits a maximum density at least 5 times the maximum 55 density obtained when an identical test layer of the said silver halide emulsion is equally exposed and then developed for 4 min. at 20° C. in the above "surface" developer.

Silver halide emulsions that meet the above requirement 60 and hence are suitable for being employed in the process of the invention are generally not or only slightly chemically ripened silver halide emulsions, since the extent of the surface latent image-forming capability increases with the degree of chemical ripening.

65 Silver chlorobromide and silver bromide emulsions have proved to be specially suitable for the purpose of the invention. When these emulsions comprise minor amounts of silver iodide, preferably not more than 5 mole percent relative to the total amount of silver halide, they are just as well suitable.

The silver halide emulsions for use in the present process are generally gelatin silver halide emulsions. However, the gelatin may wholly or partially be replaced for instance by another protein, a hydrophilic not proteinaceous colloid or a synthetic polymeric substance applied

from an aqueous dispersion. The light-sensitive silver halide emulsions may be prepared according to all known and conventional techniques for emulsion preparation. A method according to which emulsions are prepared, and which has proved to be particularly suitable for the purpose of the invention, is the so-called conversion method according to which an emulsion of a silver salt that has a higher degree of solubility than silver bromide is converted into a silver chlorobromide or a silver bromide emulsion that occasionally contains small amounts of silver iodide. This conversion is carried out preferably very slowly for instance by several consecutive steps.

The emulsions can, if desired, be modified prior to coating by the addition of all kinds of ingredients, which are generally known in the art of emulsion preparation and some of which will be set out specifically hereinafter.

Among the said ingredients may first be mentioned the common additives, for light-sensitive silver halide material such as hardening agents e.g. formaldehyde, 20 coating aids, e.g. saponine, plasticizers, e.g. glycerol, optical sensitizers of the class of the cyanine dyes, the merocyanine dyes, etc., development accelerators, compounds that render the material more resistant to wrinkling and less brittle etc.

Furthermore specific ingredients may be incorporated also. Among these may be mentioned more particularly:

Thiocyanates, such as potassium thiocyanate, which further stabilise the light-developed image;

Compounds or mixtures of compounds reducing the background density on latensification e.g. lead salts, and preferably cadmium salts; these salts are preferably salts that are water-soluble such as lead acetate, lead iodide, lead nitrate, cadmium iodide, cadmium chloride, cadmium bromide, cadmium nitrate, etc.; they give rise to a decrease of the minimum density without, however, decreasing the maximum density to the same extent so that as a result thereof the contrast is enhanced. Said salts may be added to the emulsion during the emulsion preparation or the conversion of the silver salt emulsion by means of a bromide as well as just before coating the emulsion on a support. They are added in amounts varying from about 1 g. to about 20 g., preferably from about 5 g. to about 15 g. per mole of silver halide.

The amount of gelatin applied in emulsion making is preferably such that per kg. of emulsion ready for coating from about 20 g. to about 150 g. of gelatin is present.

The amount of silver nitrate used in emulsion making preferably varies from about 50 to about 200 g. per kg. of emulsion.

The emulsion is generally coated in such a way that 1 kg. of emulsion covers approximately from about 20 to about 30 sq. m. of support.

Suitable support for the elements of this invention include the flexible supports used in the prior art for light-writing and oscillographic recording. They may be any type of paper, as well as films of cellulose nitrate, cellulose acetate, poly(vinyl acetal), polystyrene, poly(ethylene terephthalate) and other synthetic resins. Supports of glass, metal, and other substances are not excluded. In this connection conventional photographic base papers may be conveniently utilised.

In order to form an image in the light-developable radiation-sensitive photographic elements according to the present invention, said elements are first exposed to a high-intensity actinic radiation e.g. from Xenon tubes, U.V.-lamps or high-pressure mercury arc lamps as used in certain oscilloscopes.

The high-intensity radiation source used for the initial or first exposure of the light-developable material is generally rich in blue and ultraviolet radiation but said radiation may be any light or other electromagnetic radiation of either visible or invisible wave lengths, X-rays, gamma rays or an electron beam. After the initial ex-

posure the material may be light-developed by exposure to low intensity daylight, incandescent light or fluorescent light, or by the use of photoflood lamps as commonly used in photography. This secondary exposure must not necessarily be performed with the aid of an actinic radiation source. When light-developing with common office lighting or daylight the image becomes visible after 15-30 seconds, attaining maximum density in several minutes. In certain instances i.e. for obtaining practically immediately visible traces or images it may be advantageous, as already stated above, to carry out the development while supplying heat. This can be carried out by running the material over a hot plate at 80°-180° C. in the secondary exposure step.

The sharpness of the recorded trace or image may be further increased by a short preliminary exposure of the light-developable radiation-sensitive material according to the invention to ordinary light e.g. daylight, prior to exposing the material to the high-intensity radiation. Indeed, by this short preliminary exposure the gradation in the toe of the characteristic curve and the contrast or net density of the recorded trace or image are increased.

If desired the material may be chemically developed and fixed before, during or after the photo-development, 25 latensification, or secondary exposure. This development is of the internal type which means that it takes place in the presence of an energetic silver halide solubilising agent, e.g. sodium thiosulphate, which is mostly present in the developer itself. Said chemical development advantageously occurs in the presence of an anti-fogging agent. The halogen acceptor used can function as such at least when it possesses good antifogging properties. The anti-fogging agent may be incorporated in at least one of the 30 composing layers of the photographic element used and/or in the developer. Examples of suitable anti-fogging agents are 2-mercapto-ethyl-carbanilate, 1-phenyl-2-tetrazoline-5-thione and 4,5,6,7-tetrabromo-1H-benzotriazole.

It was noticed that the advantage of the chemical development of light-developable silver halide material in the presence of anti-fogging agents does not only apply to the material according to the present invention but also to any photographic material of the light-developable type.

#### EXAMPLE 1

A light-sensitive photographic silver bromide emulsion of the light-developable type, i.e. that mainly forms an internal latent image and only to a little extent an external latent image is prepared by conversion of a silver chloride emulsion into a silver bromide emulsion. Said silver bromide emulsion is prepared so that an amount of silver bromide equivalent to 120 g. (0.7 mole) of silver nitrate is present per kg. of emulsion. The usual emulsion ingredients and coating aids are incorporated into the emulsion, and in addition thereto an orthochromatic sensitizing agent, and 8 g. of cadmium bromide per kg. of emulsion for reducing the background density.

The emulsion obtained is divided into many different emulsion samples. To these samples are added the additives according to the invention as listed in the table hereinafter. The halogen-acceptor is added in an amount of 40 ccs. of a 1% by weight solution in a suitable solvent per kg. of emulsion whereas the compound setting free iodide ions, in this particular case potassium iodide, is added in an amount of 10 ccs. of a 4% by weight aqueous solution per kg. of emulsion.

All emulsion samples obtained are coated on conventional photographic paper supports such that an amount of silver halide equivalent to 4 g. of silver nitrate is present per sq. m. of light-sensitive material.

All light-sensitive materials obtained are subjected to the following identical successive treatments:

(1) They are exposed in a flash-sensitometer "Mark VI" of Edgerton, Germeshausen and Grier for 10<sup>-4</sup> sec. through a step wedge with a constant of 0.3.

(2) The exposed materials are photo-developed for 15 min. by exposure to ordinary office fluorescent lights with a total light intensity of 240 Lux whereupon the density of the image-areas and non-image areas are measured in a MacBeth reflection densitometer. The difference between the maximum and minimum density  $\Delta D$  of all materials is listed in the table hereinafter.

The number of steps of the wedge that are recorded is also listed in the table hereinafter. This number is a measure of the relative sensitivity of the different radiation-sensitive photo-developable materials.

TABLE

| Material | Additive         | $\Delta D$ | Number of steps |
|----------|------------------|------------|-----------------|
| 1        | None             | 0.12       | 6               |
| 2        | KI alone         | 0.32       | 6               |
| 3        | Compound 1 alone | 0.28       | 6               |
| 4        | Compound 1+KI    | 0.39       | 7               |
| 5        | Compound 2 alone | 0.26       | 7               |
| 6        | Compound 2+KI    | 0.36       | 7               |

As can be seen from the results listed in the above table the materials comprising potassium iodide or halogen-acceptor alone show less difference between the image and background densities than the materials comprising both potassium iodide and halogen-acceptor; thus the contrast between image and non-image areas is enhanced.

## EXAMPLE 2

A light-sensitive photographic silver bromide emulsion of the light-developable type is prepared as described in Example 1. The emulsion obtained is now divided into 3 samples A, B and C. To emulsion samples B and C is added per kg. of emulsion as anti-fogging agent 5 ccs. and 15 ccs. respectively of a 5% by weight solution in ethanol of 1-phenyl-2-tetrazoline-5-thione. To sample A no anti-fogging agent is added.

Before coating in the way as described in Example 1 each emulsion sample on a conventional photographic paper support 10 ccs. of a 2.5% by weight solution of 6,6 - dimethyl-3-thio-1,6-dihydro-as-triazine-3,5-(2H,4H)-dione in ethylene glycol monomethyl ether and 10 ccs. of a 4% by weight aqueous solution of potassium iodide are added per kg. of emulsion.

Each of the 3 materials obtained is exposed to high intensity-radiation as described in Example 1, and photo-developed by exposure for 20 min. to ordinary office fluorescent light with a total light intensity of 240 Lux.

Immediately thereafter the samples are developed at 20° C. for 1½ min. in an "internal" developer with the following composition:

Hydroquinone—6 g.  
Monomethyl-p-aminophenol sulphate—3 g.  
Sodium sulphite (anhydrous)—30 g.  
Potassium bromide—2.5 g.  
Sodium carbonate (anhydrous)—50 g.  
Sodium thiophosphate (cryst.)—10 g.  
Water to 1000 ccs.

The samples are then fixed, rinsed and dried in the usual way.

After development the image densities and background densities of each of the materials are determined and listed in the following table.

TABLE

| Sample | Maximum density | Minimum density | $\Delta D$ |
|--------|-----------------|-----------------|------------|
| A      | 1.23            | 1.16            | 0.03       |
| B      | 1.20            | 0.98            | 0.27       |
| C      | 0.63            | 0.30            | 0.32       |

From this table it appears that by the addition of an anti-fogging agent the maximum and minimum densities both decrease, the background-density, however, decreasing more markedly than the image-density. Thus, the difference between maximum and minimum density, i.e. the net density, increases when an anti-fogging agent is added.

70

12  
EXAMPLE 3

4 light-sensitive photographic silver bromide materials of the light-developable type are prepared as described in Example 1, however, without cadmium bromide and with additives according to the invention as listed in the table hereinafter. The mentioned concentrations of these additives are per kg. of emulsion ready for being coated.

All light-sensitive materials thus obtained are exposed and photo-developed for 15 min. as described in Example 1. The maximum and minimum densities are measured in a MacBeth reflection densitometer. The  $\Delta D$  values too have been listed.

| Material | Additive                                                                                       | Max. dens. | Min. dens. | $\Delta D$ |
|----------|------------------------------------------------------------------------------------------------|------------|------------|------------|
| 1        | 12.5 ccs. of a solution of 1 g. of compound 1 in 100 ccs. of ethylene glycol monomethyl ether. | 0.42       | 0.26       | 0.16       |
| 2        | 100 g. of silver iodide sol prepared as described herein.                                      | 0.69       | 0.39       | 0.30       |
| 3        | Both said additives of the materials 2 and 3 together.                                         | 0.80       | 0.43       | 0.37       |
| 4        |                                                                                                | 0.82       | 0.40       | 0.42       |

As can be seen from the above results, the materials into which halogen-acceptor or silver iodide sol alone has been incorporated show less difference between the image and background densities than the materials to which both halogen acceptor and silver iodide sol have been added. Thus, the contrast between image and non-image areas has been enhanced.

30  
We claim:

1. Photographic element comprising a radiation-sensitive silver halide emulsion layer of the light-developable type, applied from a coating composition, to which are added

- (1) at least one member selected from a silver iodide sol and a compound setting free iodide ions, and
- (2) at least one halogen acceptor corresponding to the following general formula or to a tautomeric structure thereof:



wherein each of  $\text{R}_1$ ,  $\text{R}_2$ ,  $\text{R}_3$ ,  $\text{R}_4$  and  $\text{R}_5$  is hydrogen, an 50 alkyl group or an aryl group, with the proviso, however, that at least one of the substituents  $\text{R}_2$  and  $\text{R}_3$  is hydrogen;  $\text{R}_4$  and  $\text{R}_5$  may also be the atoms necessary to complete a carbocyclic ring.

2. Photographic element according to claim 1, wherein 55 said compound setting free iodide ions is an organic or a water-soluble inorganic iodide.

3. Photographic element according to claim 2, wherein said water-soluble inorganic iodide is potassium iodide.

4. Photographic element according to claim 1, wherein 60 the silver iodide of the sol and/or the compound setting free iodide ions is (are) present in an amount of from 0.1 to 5 g. per mole of silver halide.

5. Photographic element according to claim 1, wherein 65 the halogen-acceptor corresponding to the general formula:



wherein each of  $\text{R}_1$ ,  $\text{R}_2$ ,  $\text{R}_3$ ,  $\text{R}_4$  and  $\text{R}_5$  is hydrogen, an 75 alkyl group or an aryl group, with the proviso, however,

## 13

that at least one of the substituents  $R_2$  and  $R_3$  is hydrogen;  $R_4$  and  $R_5$  may also be the atoms necessary to complete a carbocyclic ring, is present in an amount of from 0.1 to 5 g. per mole of silver halide.

6. Photographic element according to claim 1, wherein said emulsion layer is essentially a silver bromide emulsion layer.

7. Photographic element according to claim 1, wherein said emulsion layer also comprises a cadmium and/or a lead salt.

8. Photographic element according to claim 7, wherein said salt is added in an amount comprised between 5 g. and 15 g. per mole of silver halide.

9. Photographic element according to claim 1, wherein said emulsion layer also comprises a thiocyanate.

10. Photographic element according to claim 9, wherein said thiocyanate is potassium thiocyanate.

11. Photographic element according to claim 1, wherein said emulsion layer also comprises an anti-fogging agent.

12. Photographic element according to claim 11, wherein said anti-fogging agent is 1-phenyl-2-tetrazoline-5-thione.

13. Photographic element according to claim 1, wherein said emulsion layer also comprises an optical sensitising agent.

14. Photographic element according to claim 1, wherein the member selected from a silver iodide sol and a compound setting free iodide ions is added to the radiation-sensitive coating composition just before coating.

15. Photographic element according to claim 1, wherein the halogen-acceptor corresponding to the general formula:



wherein each of  $R_1$ ,  $R_2$ ,  $R_3$ ,  $R_4$  and  $R_5$  is hydrogen, an alkyl group or an aryl group, with the proviso, however, that at least one of the substituents  $R_2$  and  $R_3$  is hydrogen;  $R_4$  and  $R_5$  may also be the atoms necessary to complete a carbocyclic ring, is added to the radiation-sensitive coating composition just before coating.

16. Photographic element comprising a radiation-sensitive silver halide emulsion layer of the light-

5

10

15

20

25

30

40

35

45

## 14

developable type, the silver halide grains of which contain silver iodide at their surface, wherein said emulsion layer contains at least one halogen-acceptor corresponding to the following general formula or to a tautomeric structure thereof:



wherein each of  $R_1$ ,  $R_2$ ,  $R_3$ ,  $R_4$  and  $R_5$  is hydrogen, an alkyl group or an aryl group, with the proviso, however, that at least one of the substituents  $R_2$  and  $R_3$  is hydrogen;  $R_4$  and  $R_5$  may also be the atoms necessary to complete a carbocyclic ring.

17. Process for recording traces or images comprising exposing to a high intensity actinic radiation a photographic element according to claim 1, and light-developing the latent image formed by said initial exposure by overall exposing said element to a radiation of lower intensity.

18. Process according to claim 17, wherein an "internal" development step and a fixing step are included before, during or shortly after said light-development.

19. Process according to claim 18, wherein the development step takes place in the presence of an anti-fogging agent.

20. Process according to claim 19, wherein said anti-fogging agent is 1-phenyl-2-tetrazoline-5-thione.

21. Process according to claim 17, wherein said light-development is carried out while applying heat.

22. Process according to claim 21, wherein said heat is supplied by running the element over a hot plate heated at 80-180° C.

## References Cited

## UNITED STATES PATENTS

- 3,260,605 7/1966 Sutherns ----- 96—107  
 3,287,137 11/1966 McBride ----- 96—107  
 3,367,780 2/1968 Fix et al. ----- 96—102

NORMAN G. TORCHIN, Primary Examiner

ALFONSO T. SURO PICO, Assistant Examiner

U.S. Cl. X.R.

96—66.5, 107